# EUROPEAN PATENT SPECIFICATION

(11) **EP 0 621 915 B1**
(45) Date of publication and mention of the grant of the patent: **16.04.1997**
(21) Application number: 93902618.3
(22) Date of filing: 12.01.1993
(51) Int. Cl.: D21C 9/16

(54) **BLEACHING OF CHEMICAL PULP**
BLEICHEN VON CHEMISCHEM ZELLSTOFF
BLANCHIMENT DE PATE CHIMIQUE

(30) Priority: 21.01.1992 SE 9200152
(43) Date of publication of application: 02.11.1994
(73) Proprietor: SUNDS DEFIBRATOR INDUSTRIES AKTIEBOLAG, S-851 94 Sundsvall (SE)
(72) Inventor: LINDSTRÖM, Lars-Ake, S-860 24 Alnö (SE); SJÖDIN, Lars, S-852 41 Sundsvall (SE); NORDEN, Solveig, S-860 20 Njurunda (SE); DAHL, Marten, S-852 34 Sundsvall (SE)
(74) Representative: Sundqvist, Hans
(86) International application number: SE9300012
(87) International publication number: WO9314262

(56) References cited:
- EP-A- 0 262 836
- EP-A- 0 402 335
- WO-A-91/12368
- US-A- 4 938 842
- Journal of Wood Chemistry and Technology, Volume 2, No. 3, 1982, GOERAN GELLERSTEDT et al.:Chemical Aspects of Hydrogen Peroxide Bleaching", p. 231 - p. 250

## Description

This invention relates to a method of delignifying and bleaching of sulphate pulp without using bleaching agents containing chlorine. The method comprises oxygen delignification and possibly ozone delignification of the pulp and subsequent peroxide bleaching.

The technique of bleaching chemical pulps is now developing rapidly, because the bleaching chemicals heretofore mainly used, Cl₂, C10₂, and hypochlorite, are feared to give rise to products being a risk for the environment and health.

Until now, the discussions have been concentrated on the, emissions of chlorinated organic substance to the recipient. The majority of the countries in the world have now established limit values for these emissions, which normally are measured as AOX (Adsorbable organic halogens). As a new trend, the customers require to an ever increasing degree paper with a low content of chlorinated organic substance.

Conventional bleaching with Cl₂ disappears now more and more, and Cl₂ is replaced primarily by Cl0₂. Bleaching with Cl0₂ causes substantially lower AOX-emissions to the recipient, but the amount of chlorinated substance in the pulp is affected only insignificantly.

In recent years, the use of hydrogen peroxide at the bleaching of chemical pulps has increased considerably. Hydrogen peroxide can replace part of the chlorine chemicals.

In EP-A-402 335 a method is described at which the pulp is pretreated with complexing agent under neutral conditions. By this process, coniferous sulphate pulp can be bleached with peroxide-containing bleaching agents to 70-75% ISO at about 10% pulp consistency. In order to achieve fully bleached pulp qualities with higher ISO-brightness (above 83% ISO), this process can be combined with final bleaching with Cl0₂. As a result, this final bleaching then yields emission of AOX from the bleach plant and chlorinated organic substance in the bleached pulp.

Other known methods of reducing emissions of chlorinated organic substance to the recipient are to extend the delignification further in the closed part of the mill, i.e. in the digester house and/or oxygen step.

Extended digestion with maintained pulp quality can be achieved by impregnating the chips with black liquor in the initial phase of the cook, as described in WO-A- 91/12368. This method renders it possible to digest pulp down to a kappa number of about 10 and obtain strength properties equal to or better than with pulp digested to conventional level, kappa number 25-30. Combined with oxygen delignification, kappa numbers as low as 5-6 can be obtained for further bleaching.

By combining conventional digestion, oxygen delignification and ozone bleaching in acid environment, kappa numbers lower than 10 can be obtained.

It has, however, not been possible to produce fully bleached pulp qualities without final bleaching with Cl0₂

In bleaching of mechanical pulp with hydrogen peroxide, silicate has been supplied in the peroxide step as disclosed in EP-A-262 836 and US-A-4 938 842. However, there are important differences between bleaching of chemical and mechanical pulps, primarily due to the lignin content. Thus, in chemical pulp bleaching the intention is to remove the lignin content completely. In mechanical bleaching the intention is to reduce colored (chromophore) groups in the lignin, while the lignin content is substantially maintained. Therefore, problems and their solutions are quite different in bleaching chemical and mechanical pulp, so that bleaching methods and bleaching results cannot be transferred from one type of pulp to the other.

The present invention implies, that fully bleached sulphate pulp with a brightness above 83% ISO can be made without the use of chlorine-containing bleaching agents.

At the start of the bleaching, the pulp shall have a low kappa number. This can be achieved by conventional or extended digestion followed by O₂-delignification, alternatively by conventional or extended digestion followed by O₂- and O₃-delignification. The bleaching is initiated by a pretreatment step with complexing agent for 1-60 minutes, the pulp consistency being 1-15%, the temperature 70-110°C and pH 5-7, followed by treatment with hydrogen peroxide.

The characterizing features of the invention are apparent from the attached claims.

The pulp digested and delignified with oxygen and possibly ozone according to above shall have a kappa number below 9.5. This can be achieved by known methods of digestion and delignification. The pulp shall thereafter be pretreated with complexing agent, for example EDTA or DTPA, at a pulp consistency of 1-15% for 1-60 minutes, preferably 5-30 minutes. The temperature shall be 70-100°C, preferably 80-100°C, and the pH-value 5-7.

The pulp thus pretreated is washed and dewatered to a consistency of 18-40%, preferably 20-30%. The pH-value is increased to alkaline level, and peroxide is added together with silicate, for example sodium silicate, alternatively together with an organic complexing agent of the type phosphonic or carboxylic acid. The dwell time of the pulp in this peroxide step shall be 1/2-5 hours, preferably 1-4 hours, and the temperature 70-110°C, preferably 80-100°C. The silicate charge shall be 2-30 kg/ton pulp, preferably 5-15 kg/ton pulp, expressed as SiO₂. Alternatively, the charge of the organic complexing agent shall be 0.5-5 kg/ton pulp.

Fig. 1 is a diagram, in which the brightness of the pulp is plotted as a function of the pulp consistency at the peroxide bleaching, partly at conventional peroxide bleaching and partly at bleaching according to the invention. The starting pulp was oxygen-delignified coniferous wood sulphate pulp with kappa number 6.5 (10.5 after digestion). Curve 1 shows conventional peroxide bleaching, with a consumption of H₂O₂ of 20 kg/ton pulp. Curve 2 and, respectively, 3 refer to bleaching according to the invention with silicate addition and a consumption of H₂O₂ of 20 and, respetively, 30 kg/ton pulp.

It appears from the diagram how the brightness, after bleaching according to the invention and, respectively, after conventional bleaching, depends on the pulp consistency. At about 12% pulp consistency, the brightness obtained is equal in both cases, but at increased pulp consistency in the peroxide step an increased brightness is obtained according to the invention, while conventional peroxide bleaching results in a deteriorated brightness.

The following exemples have the object to additionally elucidate the invention and its advantages.

### EXAMPLE 1

An oxygen-delignified coniferous wood sulphate pulp (Scandinavian fir/pine) with kappa number 6.4 (10.5 after digestion according to above WO-A- 91/12368), brightness 43% ISO, intrinsic viscosity 605 dm³/kg, was pretreated with complexing agent and peroxide bleached according to the invention.

### Pretreatment

| | | |
|---|---|---|
| Pulp consistency | % | 5 |
| Time | min. | 15 |
| Temperature | °C | 90 |
| EDTA | kg/ton | 2 |
| Final pH | | 6.1 |

### Peroxide step

| | | | |
|---|---|---|---|
| Pulp consistency | % | 25 | |
| Time | min. | 240 | |
| Temperature | °C | 90 | |
| SiO₂ | kg/ton | 10 | |
| H₂O₂ consumption | kg/ton | 13.5 | 32.0 |
| Final pH | | 10.2 | 10.3 |
| Brightness | % ISO | 79.6 | 84.2 |
| Intrinsic viscosity | dm³/kg | 520 | 447 |

### EXAMPLE 2

A coniferous wood sulphate pulp with kappa number 13.3 (digested of Scandinavian fir/pine according to WO-A- 91/12368), oxygen delignified to kappa number 8.3 and ozone bleached in acid environment to kappa number 3.2, brightness 61% ISO, intrinsic viscosity 582 dm³/kg was pretreated and bleached according to the invention.

### Pretreatment as in Example 1

### Peroxide bleaching

| | | | | |
|---|---|---|---|---|
| Pulp consistency | % | 25 | | |
| Time | min. | 240 | | |
| Temperature | °C | 90 | | |
| SiO₂ | kg/ton | 10 | | |
| H₂O₂ consumption | kg/ton | 7.3 | 14.2 | 30.1 |
| Final pH | | 8.9 | 9.5 | 10.1 |
| Brightness | % ISO | 85.3 | 88.4 | 90.4 |
| Intrinsic viscosity | dm³/kg | 536 | 498 | 420 |

### EXAMPLE 3

An oxygen delignified coniferous wood sulphate pulp (digested of Pinus taeda according to WO-A- 91/12368) with kappa number 9.9, ozone bleached to kappa number 4.8, brightness 54.5% ISO, intrinsic viscosity 607 dm³/kg was pretreated and bleached according to the invention.

### Pretreatment as in Example 1

### Peroxide bleaching

| | | | | |
|---|---|---|---|---|
| Pulp consisstency | % | 25 | | |
| Time | min. | 240 | | |
| Temperature | °C | 90 | | |
| SiO₂ | kg/ton | 10 | | |
| H₂O₂ consumption | kg/ton | 7.9 | 14.6 | 29.6 |
| Final pH | | 10.2 | 10.4 | 10.6 |
| Brightness | % ISO | 81.3 | 85.3 | 87.8 |
| Intrinsic viscosity | dm³/kg | 570 | 534 | 459 |

### EXAMPLE 4

An oxygen delignified birch sulphate pulp with kappa number 9.0, brightness 59.4% ISO and intrinsic viscosity 996 dm³/kg was bleached according to the invention.

### Pretreatment as in Example 1

### Peroxide bleaching

| | | | | |
|---|---|---|---|---|
| Pulp consistency | % | | 25 | |
| Time | min | | 240 | |
| Temperature | °C | | 90 | |
| SiO₂ | kg/ton | | 10 | |
| H₂O₂ consumption | kg/ton | 8.5 | 17.5 | 35 |
| Final pH | | 10.2 | 10.4 | 10.5 |
| Brightness | % ISO | 82.2 | 85.5 | 86.5 |
| Intrinsic viscosity | dm³/kg | 903 | 975 | 822 |

The invention is not restricted to the embodiments set forth above, but can be varied within the scope of the claims.

## Claims

1. A method of delignifying and bleaching sulphate pulp without using chlorine-containing bleaching agents, comprising oxygen delignification and possibly ozone delignification of the pulp and subsequent peroxide bleaching wherein the pulp directly after the delignification is pretreated with complexing agent for 1-60 minutes, the pulp consistency being 1-15%, the temperature 70-110°C and pH 5-7, and the pulp thus pretreated is washed,
**characterized** in that the delignification is made to a kappa number below 9.5 and that the pulp after the washing is dewatered to a consistency of 18-40% and thereafter peroxide bleached in alkaline environment in the presence of silicate or an organic complexing agent of the type phosphonic or carboxylic acid.

2. A method as defined in claim 1,
**characterized** in that the peroxide bleaching is carried out for 1/2-5 hours at the temperature 70-110°C.

3. A method as defined in claim 1 or 2,
**characterized** in that as complexing agent at the pretreatment EDTA or DTPA is used.

4. A method as defined in any one of the preceding claims, **characterized** in that at the peroxide bleaching silicate is added in an amount of 2-30 kg/ton pulp, expressed as SiO₂.

5. A method as defined in any on of the claims 1-3, **characterized** in that at the peroxide bleaching an organic complexing agent of the type phosphonic acid or carboxylic acid is added in an amount of 0.5-5 kg/ton pulp

6. A method as defined in any one of the preceding claims, **characterized** in that the bleaching is carried out to a brightness exceeding 83% ISO.

## Patentansprüche

1. Verfahren zur Delignifizierung und zum Bleichen von Sulfatzellstoff ohne Verwendung von chlorhaltigen Bleichmitteln, umfassend Sauerstoff-Delignifizierung und gegebenenfalls Ozon-Delignifizierung des Zellstoffs und anschließend Peroxidbleichen, wobei der Zellstoff direkt nach der Delignifizierung mit Komplexierungsmittel 1-60 Minuten vorbehandelt wird und wobei die Zellstoffdichte 1-15%, die Temperatur 70-110°C und der pH-Wert 5-7 betragen und der so vorbehandelte Zellstoff gewaschen wird, dadurch gekennzeichnet, daß die Delignifizierung bis zu einer Kappazahl unter 9,5 ausgeführt wird und daß der Zellstoff nach dem Waschen zu einer Stoffdichte von 18-40% entwässert wird und danach in alkalischem Milieu in Gegenwart von Silicat oder einem organischen Komplexierungsmittel vom Typ Phosphon- oder Carbonsäure gebleicht wird.

2. Verfahren nach Anspruch 1, dadurch gekennzeichnet, daß das Peroxidbleichen 1/2-5 Stunden bei der Temperatur 70-110°C ausgeführt wird.

3. Verfahren nach Anspruch 1 oder 2, dadurch gekennzeichnet, daß als Komplexierungsmittel bei der Vorbehandlung EDTA oder DTPA verwendet wird.

4. Verfahren nach einem der vorangehenden Ansprüche, dadurch gekennzeichnet, daß beim Peroxidbleichen Silicat in einer Menge von 2-30 kg/t Zellstoff, ausgedrückt als SiO₂, zugegeben wird.

5. Verfahren nach einem der Ansprüche 1-3, dadurch gekennzeichnet, daß beim Peroxidbleichen ein organisches Komplexierungsmittel vom Typ Phosphonsäure oder Carbonsäure in einer Menge von 0,5-5 kg/t Zellstoff zugegeben wird.

6. Verfahren nach einem der vorangehenden Ansprüche, dadurch gekennzeichnet, daß das Bleichen bis zu einem Weißgrad über 83% ISO ausgeführt wird.

## Revendications

1. Procédé de délignification et de blanchiment de pâte au sulfate sans utilisation d'agents de blanchiment contenant du chlore, comportant une délignification à l'oxygène et éventuellement une délignification à l'ozone de la pâte et un blanchiment ultérieur au péroxyde selon lequel la pâte, directement après la délignification, est prétraitée avec un agent complexant pendant 1--60 minutes, la consistance de la pâte étant 1-15%, la température 70-110°C et le pH 5-7, et la pâte ainsi prétraitée est lavée, caractérisé en ce que le délignification est effectuée jusqu'à un indice Kappa inférieur à 9.5 et en ce que la pâte, après le lavage, est épaissie jusqu'à une consistance de 18-40% et ensuite blanchie au péroxyde dans une ambiance alcaline, en présence de silicate ou d'un agent complexant organique du type acide phosphonique ou carboxylique.

2. Procédé selon la revendication 1 caractérisé en ce que le blanchiment au péroxyde est effectué pendant ½ à 5 heures à une température de 70-110°C.

3. Procédé selon la revendication 1 ou 2 caractérisé en ce que l'on utilise comme agent complexant lors du prétraitement, l'EDTA ou le DTPA.

4. Procédé selon l'une quelconque des revendications précédentes caractérisé en ce que, lors du blanchiment au péroxyde, on ajoute du silicate en une quantité de 2-30 Kg/tonne de pâte, exprimée en SiO_{2.}

5. Procédé selon l'une quelconque des revendications 1-3, caractérisé en ce que, lors du blanchiment au péroxyde, on ajoute un agent complexant organique du type acide phosphonique ou acide carboxylique, en une quantité de 0,5-5 kg/tonne de pâte.

6. Procédé selon l'une quelconque des revendications précédentes caractérisé en ce que le blanchiment est effectué jusqu'à obtenir une blancheur dépassant 83% ISO.
